

June 21, 1949.

A. W. LIGER  
COMPOSITION FOR AND METHOD OF  
ELECTRODEPOSITION OF LEAD  
Filed Oct. 11, 1943

2,474,092



FIG. 1



FIG. 2

INVENTOR.  
ANDREW W. LIGER  
BY *Arthur M. Kahn*  
ATTORNEY

## UNITED STATES PATENT OFFICE

2,474,092

COMPOSITION FOR AND METHOD OF  
ELECTRODEPOSITION OF LEAD

Andrew W. Liger, Westboro, Mass., assignor, by  
mesne assignments, to Battelle Development  
Corporation, Columbus, Ohio, a corporation of  
Delaware

Application October 11, 1943, Serial No. 505,824

5 Claims. (Cl. 204—53)

1

My invention relates to a method and an electrolyte for the electrodeposition of lead. More particularly, it pertains to an alkaline lead plating bath and to a method of depositing lead therefrom.

The electrodeposition of lead has interesting applications for the production of corrosion resistant coatings on other basis metals and also for lead refining. For each of these uses, a dense, adherent, fine-grained lead deposit is desired. Of all the baths proposed in the prior art for the electrodeposition of lead, only two have attained any wide-spread commercial use—the fluoborate and the fluosilicate.

The fluosilicate bath is more or less standard in electrolytic lead refining, while the fluoborate bath is usually preferred in plating lead on steel and other metals. A recent development in the art of lead plating, comprising a sulfamate bath, is described in United States Patent No. 2,318,592. Although these electrolytes are capable of producing lead deposits that are satisfactory for most purposes, they still leave much to be desired from a commercial viewpoint.

Inasmuch as all three of the above-mentioned solutions are distinctly acid, special handling equipment such as glass-, lead-, or rubber-lined tanks, pumps, and pipes are required. In addition, these acid solutions constitute an industrial hazard to the personnel working with them. The fluosilicate bath is difficult to prepare for small-scale plating operations; it is subject to decomposition, forming silica and lead fluoride; and it does not give satisfactory plates directly on steel, but requires an intermediate copper deposit between the steel and the lead. The fluoborate bath gives slightly better deposits than does the fluosilicate and is more stable.

Numerous attempts have been made, and are recorded in the prior art, to develop an alkaline lead plating bath which would be relatively non-corrosive toward inexpensive iron and steel plating equipment. The plates obtained from these baths, however, tend to be spongy and non-adherent and the baths lack the necessary stability; therefore, they have failed to attain any wide-spread commercial use in spite of the desirability of eliminating the corrosiveness of the acid baths.

It is, therefore, one object of my invention to provide a method of depositing dense, adherent, fine-grained lead electroplates from an alkaline lead plating bath.

Another object of my invention is to develop a relatively non-corrosive electrolyte suitable for use in the electroplating and electrorefining of lead.

2

A further object of my invention is to provide a method of depositing dense, adherent, fine-grained lead electroplates which permits the use of ordinary steel or cast iron equipment to handle the necessary plating solution.

Still another object of my invention is to provide an alkaline electrolyte for the deposition of lead, which is capable of operation at high anode and cathode efficiencies and at low cell voltages.

10 Still a further object of my invention is to develop an alkaline lead plating bath that is stable over relatively long periods of use, economical, non-corrosive, and easy to prepare.

Various other objects of my invention will be apparent from the following description.

In the drawing,

Figure 1 is a diagram showing the effect of both agitation and bath temperature on the maximum current density practical for the production of good lead deposits from my alkaline lead electrolyte.

Fig. 2 is a view partly in elevation and partly in section illustrating the shape of the specimen used to compare the throwing power of my alkaline lead bath with the lead plating baths in use in the prior art. In this figure, the reference symbols A, B, C, D, E, F, and G indicate the location of measurements to determine the thickness of the lead deposits.

25 30 I have discovered that satisfactory, fine-grained, adherent lead electrodeposits can be obtained from an alkaline bath if the lead is present in the form of a suitable complex and if an addition agent is present to refine the grain of the electrodeposited metal and to increase the adherence of the plate to the basis metal. A distinct advantage of my process is that it is not critical in regard to composition limits of the electrolyte or to operating characteristics.

35 40 I have found that lead electrodeposits having the desired characteristics can be obtained from a bath having a composition within the following range:

|                  | Grams per liter |
|------------------|-----------------|
| Lead             | 30 to 95        |
| Rochelle salts   | 20 to 75        |
| Sodium hydroxide | 90 to 360       |
| Addition agent   | 0.2 to 1.5      |

50 55 In general, in the absence of a relatively high degree of bath agitation, I prefer to operate at a current density of from 20 to 30 amperes per square foot. However, current densities as low as 5 amperes per square foot may be used, and, as is hereinafter disclosed, much greater current

densities, for example 400 to 500 amperes per square foot or even higher, may be preferred for certain applications if sufficient bath agitation is provided. For most work I prefer to employ a bath temperature of between 140° and 190° F. However, under certain conditions, temperatures of from 125° F., or lower, up to approximately the boiling point of the solution may be used.

The lead may be added in any soluble form and preferably in the plumbous state. Basic lead carbonate is readily soluble; litharge, PbO, is satisfactory but somewhat more difficultly soluble than the basic lead carbonate. Commercial white lead also may be used, but this material is not quite so readily soluble as the relatively pure basic lead carbonate. Red lead oxide, Pb<sub>2</sub>O<sub>3</sub>, is not soluble in the bath. A concentration of 95 grams per liter represents about the upper limit of lead in the bath consistent with good plating practice. Amounts greatly in excess of this value tend to precipitate out when the bath is allowed to stand idle for a period of time. As the lead content of the bath is decreased, the tendency to form trees at high current densities increases. In order to obtain satisfactory plates at current densities in excess of 20 amperes per square foot, the lead concentration should be above approximately 30 grams per liter of bath. The lead content of the bath remains constant at the original composition, inasmuch as the maintenance lead is supplied by the anodes which dissolve at approximately 100 per cent efficiency during bath operation.

Sodium potassium tartrate (Rochelle salt), or a similar compound, is effective in maintaining the lead in solution. In place of the tartrate, other salts of aliphatic hydroxy carboxylic acids, such as citrates, malates, gluconates, lactates, and glycolates, may be used. Equivalent amounts of the respective acids, themselves, may be added in place of their salts, provided their neutralization effect is offset by alkali additions to secure proper free alkali concentration. In the case of the Rochelle salt, there is some tendency for lead to precipitate out of the bath during idle periods if less than about 20 grams of the tartrate per liter of the bath is present. Amounts in excess of this concentration appear to have no effect on the character of the plate; however, for economic reasons, I prefer to add not more than approximately 75 grams per liter of bath. Equivalent concentrations of the other aliphatic hydroxy organic acids may be used to aid in chemically

stabilizing the bath. Monocarboxylic acids, such as gluconic acid, or their salts, tend to require the use of a relatively high lead concentration as for example between 60 and 95 grams per liter of bath for best results. The use of polycarboxylic acids, such as tartaric or citric, or the salts thereof, appears to have an added advantage in my electrolyte in that they seem to increase the speed of solution of the lead; the monocarboxylic acids do not appear to be effective in this latter respect. An excess of alkali over that required to dissolve the lead is desirable. While, for economic reasons, I prefer to use sodium hydroxide, equivalent amounts of other alkalies, such as potassium hydroxide, may be used. In the case of sodium hydroxide, a concentration of at least approximately 90 grams per liter of bath is preferable. As is the case with the aliphatic hydroxy-carboxylic acids or the salts thereof, larger additions may be made without effecting the character of the plate; however, no advantages are gained by exceeding approximately 360 grams per liter.

The concentration and composition of the addition agent also can vary over relatively wide limits. In general, I prefer to use from about 0.2 to approximately 1.5 grams per liter of bath of an alkaline-stable, organic, surface active agent. Such agents as Du Pont RH556 and Du Pont TLF41, both available to the trade from E. I. du Pont de Nemours and Company, and stearyl trimethyl ammonium bromide are applicable to my improved alkaline lead plating bath. Triethanolamine is also quite effective. Betaines, or their derivatives, having the general formula



where R<sub>1</sub> is selected from the group consisting of hydrogen and alkyl radicals, and R<sub>2</sub>, R<sub>3</sub>, and R<sub>4</sub> represent alkyl radicals which may contain substituents such as hydroxyl groups; are alkaline-stable, surface active agents which are particularly applicable to my present invention. The maximum length of the alkyl radicals is limited only by the stability of the resulting compound. The data in Table I show the effect produced on the character of the plate by the addition of some of the agents I have found to be applicable to my alkaline lead bath. These tests were conducted by adding the indicated amounts of the various addition agents to an electrolyte of the following composition:

TABLE I  
Character of plate as affected by various addition agents in alkaline lead bath

| Test No. | Addition Agent                      |                      | Plating Time, Minutes | Agitation, Ft./min. | Character of Deposit                        |
|----------|-------------------------------------|----------------------|-----------------------|---------------------|---------------------------------------------|
|          | Type                                | Concentration, G./l. |                       |                     |                                             |
| 1        | None                                | 0                    | 3                     | 10.9                | Coarsely crystalline, non-adherent.         |
| 2        | du Pont RH556                       | 0.3                  | 20                    | 0                   | Good deposit.                               |
| 3        | do                                  | 0.6                  | 20                    | 26.7                | Smooth, lustrous, adherent deposit.         |
| 4        | du Pont TLF 41                      | 0.05                 | 5                     | 14.3                | Lustrous, non-adherent, some treeing.       |
| 5        | do                                  | 0.3                  | 21                    | 14.3                | Lustrous, adherent, no trees.               |
| 6        | do                                  | 0.7                  | 20                    | 14.3                | Good deposit.                               |
| 7        | Triethanolamine                     | 0.5                  | 20                    | 26.7                | Smooth, lustrous deposit, some trees.       |
| 8        | do                                  | 1.0                  | 20                    | 26.7                | Smooth, lustrous deposit, no trees.         |
| 9        | Stearyl-trimethyl-ammonium-bromide  | 0.4                  | 20                    | 26.7                | Smooth; adherent, slightly coarser than #2. |
| 10       |                                     | 1.0                  | 20                    | 26.7                | Same as #9.                                 |
| 11       | Betaine Hydrochloride               | 0.4                  | 20                    | 26.7                | Adherent deposit, slightly coarser than #2. |
| 12       | do                                  | 1.2                  | 20                    | 26.7                | Bright, smooth, adherent deposit.           |
| 13       | N-trimethyl-C-n-butyl-a-betaine     | 0.5                  | 20                    | 26.7                | Smooth adherent, slight porosity.           |
| 14       |                                     | 1.0                  | 20                    | 26.7                | Same as #13, but less porosity.             |
| 15       | N-diethylmethyl-C-n-butyl-a-betaine | 0.5                  | 20                    | 26.7                | Very fine grained, adherent deposit.        |
| 16       |                                     | 1.0                  | 20                    | 26.7                | Same as #15.                                |
| 17       | N-lauryl dimethyl-a-betaine         | 0.5                  | 20                    | 26.7                | Smooth, adherent, finer grain than #2.      |
| 18       |                                     | 1.0                  | 20                    | 26.7                | Same as #17.                                |
| 19       | N-trihydroxyethyl-C-decyt-a-betaine | 0.5                  | 20                    | 26.7                | Similar to #17, with slight pitting.        |
| 20       |                                     | 1.0                  | 20                    | 26.7                | Same as #19, but less pitting.              |

Basic lead carbonate, 75 g./l.; Sodium hydroxide, 180 g./l.; and Rochelle salt, 35 g./l. The resulting baths were operated at a current density of 20 amperes per square foot and at a temperature of from 160° to 165° F. Other compounds, such as N-trimethyl-C-decyl-a-betaine, N-dimethyl-ethyl-C-decyl-a-betaine, N-diethylmethyl-C-decyl-a-betaine, N-trimethyl-C-cetyl-a-betaine, N-diethyllauryl-a-betaine, and N-triethyl-C-decyl-a-betaine, are also effective addition agents for use in connection with my invention. When less than about 0.2 gram of the addition agent is present per liter of the bath, the plates tend to be dark, coarsely crystalline, porous, and non-adherent. When more than about 0.2 gram per liter is present, the resultant plate is finely crystalline, semi-lustrous, and thoroughly adherent. Amounts in excess of approximately 1.5 grams per liter are not economic, and, in some cases, the agent tends to separate from the bath in the form of an emulsion. Although additions in excess of 1.5 grams per liter appear to have little advantage, additions up to the point of separation as an emulsion may be made. In some instances the character of the deposit may be further improved by the addition of small amounts, for example from 0.5 to 2.0 grams per liter, of a wetting agent, such as Duponol ME a sulfonated lauryl alcohol.

Although the alkaline lead plating bath of my invention may be prepared in any suitable and convenient manner, I have found the following procedure to be adequate: About 75 per cent of the final volume of water is introduced into a suitable container and the required amount of alkali is added in small increments with continuous stirring. This addition tends to cause an increase in temperature. The required amount of aliphatic hydroxy carboxylic acid, or of its salt, is then added to the solution, again with continuous stirring. The requisite amount of lead, as basic lead carbonate or other soluble lead compound, is added in small lots, keeping the temperature of the solution above 180° F. and maintaining continuous agitation. When the lead is all in solution, the bath is cooled, filtered to remove any lead that is oxidized to red lead oxide or other insoluble material, diluted to the proper volume, and the required amount of the addition agent added.

As mentioned hereinbefore, my alkaline lead plating bath can be operated over a rather wide range of current densities and temperatures. As is clearly shown in Figure 1 of the drawing, the maximum current density practical for the production of good plates increases as the temperature of the bath and the amount of bath agitation increase. Under the conditions shown in Figure 1, representing those of relatively quiet bath operation, the maximum current densities permitting the production of good electrodeposits vary from about 5 to 50 amperes per square foot, depending upon the bath temperature. Under conditions of more violent agitation, much higher current densities may be used. Under the latter conditions, current densities of 500 amperes per square foot or higher are entirely practical. The data for Figure 1 were obtained from an electrolyte of the following composition: Basic lead carbonate, 75 g./l.; sodium hydroxide, 180 g./l.; Rochelle salt, 35 g./l.; and Du Pont RH556, 0.3 to 0.7 g./l.

Data comparing cell voltage measurements for my hereindisclosed alkaline lead bath with those for two commercial acid baths are given in Table II. Identical anodes and electrical arrangements

were used for each test. The commercial baths were operated according to the best available data. Anode area, anode spacing, and cathode area and material were also the same in each run. 5 All plates were made directly on plain, low-carbon steel. The data recorded in Table II show that the operating tank voltage of my alkaline lead bath is about one-third that of the fluoborate bath and only about one-fourth that of the sulfamate bath. Since the anode and cathode efficiencies of all three baths are close to 100 per cent, the lower cell voltage of my alkaline bath results in a lower power cost per unit weight of lead deposited. As shown by the data in Table 10 III, the desirably low cell voltages are obtained in electrolytes having other compositions within the scope of my present invention. All of the tests recorded in Table III were made using a current density of 20 amperes per square foot.

TABLE II

Comparative cell voltage data<sup>1</sup>

| Test No.                                     | Cell Current, Amperes | Current Density, Amps. per sq. ft. | Cell Voltage | Remarks                           |
|----------------------------------------------|-----------------------|------------------------------------|--------------|-----------------------------------|
| ALKALINE LEAD BATH (1)—TEMPERATURE 165° F.   |                       |                                    |              |                                   |
| 21-----                                      | 1.01                  | 20                                 | 0.125        | Good Deposit, finely crystalline. |
| 22-----                                      | 1.00                  | 20                                 | 0.110        | Do.                               |
| FLUOBORATE BATH (2)—TEMPERATURE 75° F.       |                       |                                    |              |                                   |
| 23-----                                      | 1.01                  | 20                                 | 0.34         | Good Deposit, finely crystalline. |
| 24-----                                      | 1.00                  | 20                                 | 0.35         | Do.                               |
| SULFAMATE BATH (3)—TEMPERATURE 75° F.        |                       |                                    |              |                                   |
| 25-----                                      | 1.00                  | 20                                 | 0.48         | Good Deposit, finely crystalline. |
| 26-----                                      | 1.00                  | 20                                 | 0.50         | Do.                               |
| 1 Composition of baths: (1) Grains per liter |                       |                                    |              |                                   |
| Basic lead carbonate.....                    |                       |                                    |              | 75                                |
| Sodium hydroxide.....                        |                       |                                    |              | 180                               |
| Rochelle salt.....                           |                       |                                    |              | 35                                |
| Du Pont RH556.....                           |                       |                                    |              | 0.5-0.7                           |
| (2)                                          |                       |                                    |              |                                   |
| Basic lead carbonate.....                    |                       |                                    |              | 150                               |
| 50% hydrofluoric acid.....                   |                       |                                    |              | 240                               |
| Boric acid.....                              |                       |                                    |              | 106                               |
| Animal glue.....                             |                       |                                    |              | 0.2                               |
| (3)                                          |                       |                                    |              |                                   |
| Du Pont lead sulfamate salt.....             |                       |                                    |              | 355                               |
| Du Pont addition agent #1.....               |                       |                                    |              | 9.72                              |

TABLE III

## Cell voltage data for other alkaline lead baths

| Test No. | Bath <sup>1</sup> No. | Cell Voltage | Bath Temperature, °F. | Remarks                        |
|----------|-----------------------|--------------|-----------------------|--------------------------------|
| 27-----  | 1                     | 0.12         | 150                   | Smooth, lustrous deposit.      |
| 28-----  | 2                     | 0.12         | 150                   | Slightly coarser than #27.     |
| 29-----  | 3                     | 0.15         | 162                   | Similar to #28, some treeling. |
| 30-----  | 4                     | 0.15         | 160                   | Slightly rough.                |
| 31-----  | 5                     | 0.10         | 163                   | Very lustrous, few pits.       |
| 32-----  | 6                     | 0.20         | 100                   | Slightly rough.                |
| 33-----  | 6                     | 0.08         | 164                   | Smooth and lustrous.           |

<sup>1</sup> Bath compositions:

1. 50 g./l. basic lead carbonate, 180 g./l. sodium hydroxide, 20 g./l. lactic acid, 0.2 g./l. Du Pont RH556.
2. 50 g./l. basic lead carbonate, 180 g./l. sodium hydroxide, 40 g./l. lactic acid, 0.2 g./l. Du Pont RH556.
3. 50 g./l. basic lead carbonate, 180 g./l. sodium hydroxide, 60 g./l. lactic acid, 0.2 g./l. Du Pont RH556.
4. 50 g./l. basic lead carbonate, 180 g./l. sodium hydroxide, 20 g./l. gluconic acid, 0.6 g./l. Du Pont RH556.
5. 94 g./l. basic lead carbonate, 360 g./l. sodium hydroxide, 40 g./l. gluconic acid, 0.6 g./l. Du Pont RH556.
6. 94 g./l. basic lead carbonate, 360 g./l. sodium hydroxide, 20 g./l. lactic acid, 0.2 g./l. Du Pont RH556.

A further advantage of my alkaline lead bath is its relatively high throwing power. Comparison tests of throwing power were made in the

that carbon additions up to a maximum of at least 55 grams per liter have no deleterious effects on the deposited metal or on the bath operation.

TABLE IV  
Comparative throwing power data<sup>1</sup>

| Test No.                               | Current Density, Amps. per sq. ft. | Plating Time, Minutes | Thickness of Lead Deposit in Inches at Position <sup>2</sup> |         |         |         |         |         |         |
|----------------------------------------|------------------------------------|-----------------------|--------------------------------------------------------------|---------|---------|---------|---------|---------|---------|
|                                        |                                    |                       | A                                                            | B       | C       | D       | E       | F       | G       |
| ALKALINE LEAD BATH—TEMPERATURE 165° F. |                                    |                       |                                                              |         |         |         |         |         |         |
| 34.....                                | 14                                 | 20                    | 0.00105                                                      | 0.0010  | 0.00045 | 0.00021 | 0.00029 | 0.00075 | 0.00190 |
| FLUOBORATE BATH—TEMPERATURE 75° F.     |                                    |                       |                                                              |         |         |         |         |         |         |
| 35.....                                | 20                                 | 20                    | 0.00085                                                      | 0.00085 | 0.00000 | 0.00000 | 0.00000 | 0.00060 | 0.00135 |
| SULFAMATE BATH—TEMPERATURE 75° F.      |                                    |                       |                                                              |         |         |         |         |         |         |
| 36.....                                | 20                                 | 21                    | 0.00175                                                      | 0.00025 | 0.00018 | 0.00017 | 0.00015 | 0.00055 | 0.00210 |

<sup>1</sup> Bath compositions shown in Table II.

<sup>2</sup> Position on specimen as indicated by Figure 2.

three bath compositions recorded in Table II. For these tests, strips of plain, low-carbon steel 6 1/4 inches long and 1 inch wide were bent into a narrow U shape as shown in Figure 2 of the drawing. Specimens of this type were then plated, under the commercially preferred conditions, in each of the three electrolytes noted in Table II. In conducting these tests, the specimens were immersed in the respective baths in such a manner that 5 inches of the total length was plated. The specimens were positioned with the long axis of the U parallel to the surface of the bath, and anodes were placed on the extension of the long axis approximately 1/2 inch from the open and the closed ends of the U. After plating, the thickness of the lead electroplate was determined at the locations designated by the reference symbols A, B, C, D, E, F, and G of Figure 2. These measurements were made along the central axis of the specimen. The data in Table IV show the results of these tests. By dividing the plate thickness at D by the average plate thickness at A and G and multiplying the result by 100, values for the throwing power of the respective baths may be obtained. On this basis, the throwing power of my alkaline lead bath is indicated to be 14 per cent of the ideal, while the sulfamate and the fluoborate baths have values of 8.85 per cent and 0.0 per cent of the ideal, respectively. In other words, my alkaline bath is superior in throwing power to either the sulfamate or the fluoborate baths. In addition, the plates from the alkaline bath showed less tendency to tree on some of the higher current density points.

The alkaline bath of my invention has an excellent operable life. Although the addition agent must be replaced from time to time, the consumption of the agent is quite low. For example, in the case of Du Pont RH556, the apparent consumption is approximately 0.01 gram per liter per ampere-hour of use. Inasmuch as a relatively large portion of the loss occurs through mechanical dragout, the true addition agent consumption is actually well under the above-mentioned figure.

Over relatively long periods of operation, the alkaline bath tends to pick up carbon dioxide from the atmosphere, forming alkali carbonate in the bath. However, actual tests have shown

In general, the electrodeposits from my alkaline bath have been investigated and compare favorably with plates from acid-type baths in regard to porosity, atmospheric corrosion resistance with and without a copper undercoat, resistance to chemical attack, adherence and solderability.

It can be seen from the above that I have developed a new and novel electrolyte and method for the electrodeposition, electroforming, and electrorefining of lead. Lead deposited by means of my invention is dense, adherent, and fine-grained. The electrolyte is relatively non-corrosive to iron and steel equipment or to any other materials commonly used for alkaline baths, such as glass, wood and certain types of rubber; it operates at low cell voltages; it is stable over long periods of use; and it has a relatively high throwing power. The lead deposits from the disclosed electrolyte are satisfactory for use in the well-known applications of lead plating.

While specific examples have been given in the foregoing specification, these examples are given merely to illustrate the principles of my invention, and the invention is not limited to or by such examples.

Having thus described my invention, what I claim is:

1. An alkaline electrolyte suitable for the deposition of dense, adherent lead electrodeposits, said electrolyte containing from 30 to 95 grams per liter of dissolved lead, from 20 to 75 grams per liter of a salt of an aliphatic hydroxy carboxylic acid, alkali equivalent to from 90 to 360 grams per liter of sodium hydroxide, and from 0.2 to 1.5 grams per liter of a betaine, the balance of said electrolyte being primarily water.

2. An alkaline electrolyte suitable for the deposition of dense, adherent lead electrodeposits, said electrolyte containing from 30 to 95 grams per liter of dissolved lead, from 20 to 75 grams per liter of a salt of tartaric acid, alkali equivalent to from 90 to 360 grams per liter of sodium hydroxide, and from 0.2 to 1.5 grams per liter of a betaine, the balance of said electrolyte being primarily water.

3. An alkaline electrolyte suitable for the deposition of dense, adherent lead electrodeposits, said electrolyte containing from 30 to 95 grams per liter of dissolved lead, from 20 to 75 grams

per liter of a salt of citric acid, alkali equivalent to from 90 to 360 grams per liter of sodium hydroxide, and from 0.2 to 1.5 grams per liter of a betaine, the balance of said electrolyte being primarily water.

4. The method of producing dense, adherent lead electrodeposits which comprises making the article to be plated the cathode in an alkaline electrolyte containing from 30 to 95 grams per liter of dissolved lead, from 20 to 75 grams per liter of a salt of an aliphatic hydroxy carboxylic acid, alkali equivalent to from 90 to 360 grams per liter of sodium hydroxide, and from 0.2 to 1.5 grams per liter of a betaine, the balance of said electrolyte being primarily water, and passing an electric current therethrough of sufficient strength and for a sufficient time to produce the desired thickness of deposited lead.

5. The process which comprises electrodepositing lead from an aqueous alkaline solution containing alkali metal plumbite in concentration equivalent to about 6 oz./gal. of PbO and about

0.03 oz./gal. of a betaine selected from the group consisting of trimethyl-c-cetyl alpha-betaine, trimethyl-c-decyl alpha-betaine, and dimethyl-N-lauryl alpha-betaine.

ANDREW W. LIGER.

#### REFERENCES CITED

The following references are of record in the file of this patent:

#### UNITED STATES PATENTS

| Number    | Name             | Date          |
|-----------|------------------|---------------|
| 1,619,835 | Summers          | Mar. 8, 1927  |
| 2,048,594 | Brockman         | July 21, 1936 |
| 2,107,806 | Soderberg et al. | Feb. 8, 1938  |
| 2,255,057 | Holt             | Sept. 9, 1941 |

#### OTHER REFERENCES

- Transactions of the Electrochemical Society, vol. 23, page 175 (1913).  
 20 Transactions of the Electrochemical Society, vol. 38, page 121 (1920).

**Certificate of Correction**

Patent No. 2,474,092.

June 21, 1949.

ANDREW W. LIGER

It is hereby certified that error appears in the printed specification of the above numbered patent requiring correction as follows:

Column 8, line 1, for the word "carbon" read *carbonate*;  
and that the said Letters Patent should be read with this correction therein that the same may conform to the record of the case in the Patent Office.

Signed and sealed this 6th day of December, A. D. 1949.

[~~SEAL~~]

THOMAS F. MURPHY,  
*Assistant Commissioner of Patents.*